

## UNITED STATES PATENT OFFICE

EGON ELÖD, OF KARLSRUHE, GERMANY

## PROCESS FOR THE RECOVERY OF COCOS FIBERS

No Drawing. Application filed March 25, 1929, Serial No. 348,909, and in Germany March 27, 1928.

The cocoanut fibers usually obtainable in the trade are, as is well known, unsuitable for mechanical spinning in technical industrial establishments on account of their hardness 5 and small suppleness.

Now it has been found that such fibers can be materially improved by treatment with alkaline liquids at raised temperatures preferably at temperatures over 100° C. for example from 120 to 150° C., rapidly and at 10 relatively small cost so that they become soft and elastic while retaining their breaking or tearing strength, thus being made suitable for spinning by machinery.

For example, the raw fiber is subjected to the treatment of caustic soda solution of about 15 3% strength for twenty minutes in a closed container at a temperature of 135° C. The solution is preferably maintained in circulation 20 by means of any appropriate device.

After lixiviation and drying the fibers thus treated are soft and particularly elastic. Such fibers may for definite uses be subjected 25 to subsequent treatment with hygroscopic agents or with fat- or oil-containing substances. The alkaline liquids employed may after use be conveyed to another container and after suitable regeneration for example, by adding sufficient alkali to bring the solution 30 up to 3%, and heating be used again, enabling thereby the cost of the process to be further considerably reduced.

It has already been proposed to treat the fiber padding of cocoanuts with hot dilute 35 solutions for the recovery of the fibers. In this treatment, however, the fiber does not become soft because the alkali present is used to open up the cork-like bedding layer of the fiber padding in large quantities and is thus 40 rendered useless for softening the liberated fiber so as to make it suitable for spinning.

In accordance with this invention the novel discovery of the softening effect of alkaline liquids is utilized in that already isolated 45 fibers i. e., fibers freed from the bedding substance referred to and if need be also subjected to a cleaning process are treated with alkaline liquids in order thereby to improve the fibers more especially for spinning by machinery.

The isolation of the fiber from the bedding substance thereof may be effected by means of various methods for instance by a preliminary dipping of the shell of the cocoanut in hot water while maintaining it in motion and thereafter subjecting it to a mechanical treatment, for example crushing it, whereupon the dipping in hot water is repeated for a short time again with motion and finally the fibers may be readily separated from the bedding 55 substance by ordinary methods, for example by combing.

I claim:

1. The process of preparing soft, supple, 60 spinnable cocoanut fibers which includes subjecting hard, raw fibers freed from bedding substances to the action of a weak alkaline solution maintained at a temperature above 100° C. in a closed container, for a period of less than one hour.

2. The process of preparing soft, supple, 65 spinnable cocoanut fibers as defined in claim 1 in which the alkaline solution used is caustic soda and the time of treatment in the closed container is substantially twenty minutes.

3. The process of preparing soft, supple, 70 spinnable cocoanut fibers which includes, subjecting hard, raw fibers freed from bedding substances to the action of an alkaline solution of 2 to 3% strength maintained at a temperature above 100° C. in a closed container, for a period of less than one hour.

4. The process of preparing soft, supple, 75 spinnable cocoanut fibers which includes subjecting hard, raw fibers freed from bedding substances to the action of a weak alkaline solution maintained at a temperature of 120° C. to 150° C. in a closed container.

5. The process of preparing soft, supple, 80 spinnable cocoanut fibers which includes, subjecting hard, raw fibers freed from bedding substances to the action of an alkaline solution of 2 to 3% strength maintained at a temperature of 120° to 150° C. in a closed container.

6. The process of preparing soft, supple, 85 spinnable cocoanut fibers which includes, subjecting hard, raw fibers freed from bedding substances to the action of a weak alka- 90

55

60

70

75

80

85

90

95

100

line solution maintained at a temperature above 100° C. in a closed container and finishing the softened fiber by treating it with oleaginous finishing substances.

7. The process of preparing soft, supple, spinnable cocoanut fibers which includes, subjecting hard, raw fibers freed from bedding substances to the action of a weak caustic alkali solution maintained at a temperature above 100° C. in a closed container and finishing the softened fiber by treating it with oleaginous finishing substances.

In testimony whereof I affix my signature.

EGON ELÖD.

15

20

25

30

35

40

45

50

55

60

65